

## UNITED STATES PATENT OFFICE

2,192,832

## METHOD OF MANUFACTURING COVERED WIRES

Hidejiro Ito, Yokohama-Shi, and Takeshi  
Masuda, Tokyo-Shi, JapanNo Drawing. Application February 4, 1939, Serial  
No. 254,742. In Japan March 1, 1938

3 Claims. (Cl. 57—162)

This invention relates to an improvement in a method of manufacturing covered wires, which is simple, efficient and less expensive than the method used heretofore.

Previously in the method of covering wires with cotton or paper, a cotton thread or paper tape was wound around the wire throughout its entire length. In order to obtain a uniformly covered wire the cotton threads employed were very fine and the paper tapes employed were uniformly thin, so that it was comparatively expensive to cover the wire with a cotton thread or a paper tape. Moreover, considerable difficulty had been experienced in obtaining a uniform layer of the cover on the wire throughout its length.

The object of the present invention is to provide an improved method whereby a wire may be covered easily and uniformly at less expense.

According to the present invention, suitable vegetable fibres, crushed or broken into suitable pieces, are intermingled with a liquid, such as water, which may contain a small quantity of size or like material dissolved therein, so as to be held in suspension in said liquid. A wire to be covered is passed through the liquid containing the suspended fibres, the wire being revolved, or the liquid being whirled around the wire by any suitable means. In this manner, the fibres in suspension in the liquid are caused to wrap themselves securely and uniformly around the wire to form the desired covering. Thus, a wire may be covered with any desired vegetable fibre more compactly and uniformly in a simple operation and at less cost as compared with the methods heretofore practiced.

In carrying out the present invention a suitable vegetable fibre, such as the fibre of cotton, hemp, flax or pulp is crushed or broken into suitable pieces and then split up and loosened. Several percent by weight of the fibre is then intermingled with a liquid containing a small quantity

of *Chondrus ocellatus*, the mucus of *Hibiscus manihot* root, or the like dissolved therein, whereby a somewhat viscous solution containing the fibres in suspension is produced. For example, the solution may consist of 0.5% pulp fibre, 0.5% mucus and 99% water. A wire is passed through said solution while being revolved so that the fibre in suspension in said solution is wound around the wire. Instead of revolving the wire, the solution in the vessel may be whirled around the wire by any suitable means with the same effect. The speed with which the wire is fed into the liquid and the speed of revolution of the wire or whirling of the solution are regulated according to the desired thickness of the fibrous cover on the wire. The wire thus covered is then preferably passed through a die or rollers adjusted to the size of said covered wire in order to make the cover trim and neat.

It will be understood that the invention may be applied to the covering of any kind of wires, rods, bars, or tubes without departing from the scope of the invention.

What we claim is:

1. A method of manufacturing covered wires comprising splitting up and loosening a crushed and broken vegetable fibre, intermingling said fibre in a liquid to form a suspension, and passing the wire through said suspension while revolving said wire relatively to said liquid whereby the suspended fibre is wound quickly and uniformly around said wire.

2. A method as claimed in claim 1 wherein the vegetable fibre consists of a material selected from the group consisting of cotton, hemp, flax and pulp.

3. A method as claimed in claim 1 wherein the liquid consists of water and a small quantity of size.

HIDEJIRO ITO.  
TAKESHI MASUDA.

40